

## UNITED STATES PATENT OFFICE

VICTOR D. DAVIGNON, ATTLEBORO, MASSACHUSETTS, ASSIGNOR TO GENERAL PLATE COMPANY, OF ATTLEBORO, MASSACHUSETTS, A CORPORATION OF RHODE ISLAND

## GOLD ALLOY

No Drawing.

Application filed June 10, 1926. Serial No. 115,114.

The invention relates to alloys of precious metals, and particularly to alloys of gold containing metals of low specific gravity, and to the process of making the same.

5 The gold alloy now commonly used in the arts has as its characteristic constituents gold and copper or gold and silver with appropriate base metals other than copper or silver to impart requisite hardness, color, and other 10 desired properties. This alloy, although malleable and ductile to a degree permitting working by usual mill processes of rolling and drawing, has the disadvantage of possessing a relatively high specific gravity, and the 15 present invention has among its objects the reducing of the specific gravity of such alloys by incorporating therein a sufficient quantity of low specific gravity metal or metals such as calcium, lithium, magnesium, silicon, titanium, and aluminum for materially 20 reducing the specific gravity of the alloy.

It will be understood that small percentages of metals of low specific gravities in the order of the specific gravities of the metals 25 mentioned above will materially reduce the specific gravity of the gold alloy, which can be appreciated from an observation that in a 14 carat gold alloy containing by weight 1 part magnesium out of 24 parts alloy the 30 magnesium will have a volume about 80% that of the gold.

I have found that magnesium, calcium, lithium, and other metals of similar characteristics cannot be alloyed with gold by usual 35 processes, and that the mixture of raw metals to be compounded to make the alloy, particularly when magnesium is present, is explosive upon application of heat sufficient to raise the temperature of the mixture to a 40 value necessary to melt the gold. These effects I explain are due to the fact that such low specific gravity metals are highly volatile at temperatures much below that at which gold melts, and consequently will be destroyed 45 by high temperatures, the destruction being aided by the strong affinity of the metals for oxygen.

According to the practice of the improved process the low specific gravity metal is first 50 alloyed with a metal or metals with which it

will combine without being destroyed, the resulting alloy then being alloyed with the gold or with a gold alloy. Preferably, but not necessarily, the low specific gravity metal is alloyed with a metal which has a melting point less than that of the low specific gravity metal, so that the latter will be combined at as low a temperature as possible, and preferably, when the final product will permit, 55 other metal is incorporated to cause the resulting preliminary alloy to have a melting point higher than that of the low specific gravity metals but less than that of gold. Preferably also, but not necessarily, the gold 60 before being alloyed with the preliminary alloy is itself alloyed with a metal to produce a resulting alloy which will have a melting point less than that of gold. The low specific gravity alloy and the gold alloy may 65 then be alloyed at a temperature between that of the melting point of the low specific gravity metal and that of the gold, with the result that the final alloy may be produced without 70 at any time subjecting the raw low specific gravity metal or the alloy containing it to an unnecessarily high temperature.

As an example of the practice of the invention, but without limitation thereto, a preliminary alloy consisting of by weight about 20% magnesium, 30% zinc, and 50% silver 75 may be made by placing the raw metals in a crucible and raising their temperature to about 1400 degrees Fahrenheit, with use of suitable fluxes as hereinafter described. I have found that the zinc melts first and apparently causes the magnesium to melt into it at a temperature lower than that of the melting point of raw magnesium, and the silver to melt into the liquid zinc and magnesium at a temperature lower than that of the melting point of silver, the zinc therefore acting to reduce the melting point of the silver and magnesium. The silver makes the 80 alloy more homogeneous, and raises its melting point above that of the magnesium so that the alloy may be alloyed with gold or with a gold alloy without to any appreciable extent destroying the magnesium, which 85 would be the tendency if only magnesium and zinc were used. I have found it possible how- 90

ever to omit the silver, but without as easily securing satisfactory results. Such substitute alloy may consist of 50% magnesium and 50% zinc. It is also possible to omit the zinc and 5 still secure satisfactory results, but with greater difficulty. As an example of a substitute alloy of this nature I may use 30% magnesium and 70% silver. The magnesium 10 alloys, of which examples are given above, 15 are in the nature of chemical combinations, being brittle as glass, the silver alloys melting at about 1400 degrees Fahrenheit. These alloys have the property of causing gold when mixed with the alloy to melt at a temperature of about 1600 degrees Fahrenheit, which is lower than the melting point of gold.

In making the preliminary alloy the metals may be placed in the crucible in lump, shot, bar, or sheet form in the inverse order 20 of their specific gravities, that is to say the low specific gravity metal in the bottom of the crucible and the metals of higher specific gravity above it, so that the low specific gravity metal upon melting tends to rise through 25 the metals of high specific gravity.

I have found as suitable for flux in preparing the preliminary alloy potassium bifluoride or calcium chloride, or a mixture of the two in the proportion of 1 part calcium chloride 30 and 2 parts potassium bifluoride, cryolite, potassium chloride, sodium chloride, and sodium fluoride. The flux preferably is placed in the crucible in crystalline or powdered form on top of the metals before heat 35 is applied, sufficient flux being employed to maintain upon the molten metals a layer about  $\frac{1}{4}$  inch thick. The contents of the crucible together with the flux and slag are poured simultaneously in a thin stream into 40 the mold so at all times to protect the molten metal from the action of the air. I have found that this flux effectively will eliminate all oxides of the metals entering into the alloy, which oxides if present in the final alloy 45 will render it unhomogeneous. It will be understood that the invention is not limited to use of the fluxes given, but that other fluxes, which will eliminate the oxides of the low 50 specific gravity metal and form a liquid seal preventing access of air to the molten metal, may be employed.

The gold preferably is alloyed with the remaining constituents of the final alloy prior to being alloyed with the preliminary alloy 55 containing the volatile low specific gravity metal. For example, if the alloy to be produced is to contain gold, copper, silver and magnesium, the gold may be first alloyed with the copper and some of the silver, and 60 the magnesium is first alloyed with the zinc and balance of the silver, both of these alloys as heretofore explained having a melting point less than that of gold. These two alloys are then placed in a crucible and melted.

65 The specific gravity of the alloy to be pro-

duced may be further reduced by incorporating other low specific gravity metals, as for example aluminum which is not particularly volatile, in which case the aluminum will be preliminarily alloyed with the gold and copper, as for example by practice of the method described in United States Patent 1,557,431 granted to me October 13, 1925.

In making the final alloy the preliminary alloy containing the volatile low specific gravity metal may be placed at the bottom of the crucible and the alloy containing the gold on top of it, the two alloys being in relatively small pieces. The metals are then covered with a layer about  $\frac{1}{4}$  inch thick of suitable flux and the crucible is placed in a furnace and raised to 1600 degrees Fahrenheit, at which temperature the metals become liquid. More flux is then placed in the crucible, say about 1 ounce for each hundred troy ounces 80 of metal, and the temperature is raised to about 1700 degrees, at which temperature the crucible is removed from the furnace and the contents thereof are poured in a thin stream into the mold, which mold may have an elongated vertically inclined mold chamber of the type described in my aforesaid patent.

As suitable fluxes for making the final alloy I may use those described above in connection with the preliminary alloy. In addition I 95 have also found as suitable for use granular sodium chloride, window glass, green bottle glass, mercury bichloride, and potassium cyanide, all of which will dissolve or otherwise eliminate the oxides of the low specific gravity metals. I have found that a mixture of 75% sodium chloride, 12½% potassium fluoride, and 12 cryolite gives excellent results.

The above described process is particularly useful in connection with calcium, lithium, 105 and magnesium, and other highly volatile low specific gravity earthy metals. Less volatile low specific gravity earthy metals such as aluminum and low specific gravity ferrous metals such as silicon and titanium if desired 110 also may be alloyed with gold by the above described method.

As an example of a desirable 14 carat commercial green gold alloy the same may consist of about 58% gold, 25% silver, 3% magnesium, 5% zinc, with the remainder copper, or if desired some of the copper may be substituted by aluminum, for example to make the alloy contain 3% aluminum. As an example of a desirable commercial 14 carat yellow gold alloy the alloy may consist of about 58% gold, 3% magnesium, 5% zinc, with the remainder copper, or if desired some of the copper may be replaced by aluminum, for example enough to make the alloy contain 3% 120 aluminum.

I have found that by practice of the above method calcium in amounts up to 0.5%, lithium up to 1%, and magnesium up to 3% readily may be incorporated into the alloy.

By exercise of care it is possible to raise the calcium content up to 2%, the lithium up to 3%, and the magnesium up to 5%.

My improved alloy is distinguished from prior alloys in that it contains low specific gravity metals, particularly highly volatile earthy metals in amount sufficient materially to reduce its specific gravity, while at the same time it is sufficiently malleable and ductile to permit working thereof by the usual mill processes of alternate attenuation and annealing, the ingot being sufficiently homogeneous and free from checks and blisters to permit economic utilization thereof.

15 Although I have described several examples of alloys and metals for use therein, one example of the improved method and several examples of fluxes for use therewith, it is to be understood that within the scope of 20 my invention wide deviations may be made without departing from its spirit.

Claims—

1. A substantially homogeneous, malleable and ductile gold alloy containing by weight 25 about 58% gold, 8% copper, 3% magnesium, 5% zinc, and the remainder silver.

2. A substantially homogeneous, malleable and ductile gold alloy containing by weight about 58% gold, 3% magnesium, 5% zinc, and 30 the remainder consisting of a metal of the group comprising silver and copper.

3. A substantially homogeneous malleable and ductile gold alloy containing by weight about 58% gold, 8% copper, 3% aluminum, 35 3% magnesium, 5% zinc, and the remainder silver.

4. A substantially homogeneous malleable and ductile gold alloy containing by weight about 58% gold, 3% magnesium, 3% aluminum, 5% zinc, and the remainder consisting 40 of metal of the group comprising silver and copper.

5. A substantially homogeneous, malleable and ductile gold alloy having by weight from 45 25 to 85% gold, from 1 to 5% magnesium, the remainder predominately metal of the group comprising silver and copper.

6. A substantially homogeneous, malleable 50 and ductile gold alloy having by weight from 25 to 85% gold, from 1 to 5% magnesium, a small but substantial amount of zinc, the remainder predominately metal of the group comprising silver and copper.

55 7. A substantially homogeneous, malleable and ductile gold alloy having by weight from 25 to 85% gold, 1/2 to 5% metal of the group comprising magnesium, calcium and lithium, the remainder predominately metal of the 60 group comprising silver and copper.

8. A substantially homogeneous, malleable and ductile gold alloy having by weight from 65 25 to 85% gold, 1/2 to 5% metal of the group comprising magnesium, calcium and lithium, a small but substantial amount of zinc, the

remainder predominately metal of the group comprising silver and copper.

9. A substantially homogeneous, malleable and ductile gold alloy having by weight from 25 to 85% gold, from 1 to 5% magnesium, a 70 substantial amount of aluminum up to 3%, a small but substantial amount of zinc, the remainder predominately metal of the group comprising silver and copper.

In testimony whereof, I have signed my 75 name to this specification.

VICTOR D. DAVIGNON.